

## UNITED STATES PATENT OFFICE

2,593,431

REAGENT CONDITIONING FOR ELECTRO-  
STATIC SEPARATION OF MINERALSFoster Fraas, Riverdale, Md., assignor to the  
United States of America as represented by the  
Secretary of the Department of the InteriorNo Drawing. Application January 16, 1948,  
Serial No. 2,800

2 Claims. (Cl. 209—9)

(Granted under the act of March 3, 1883, as  
amended April 30, 1928; 370 O. G. 757)

1

The invention described herein may be manufactured and used by or for the Government of the United States for governmental purposes without the payment to me of any royalty thereon in accordance with the provisions of the act of April 30, 1928 (Ch. 460, 45 Stat. L. 487).

This invention relates to the electrostatic separation of minerals. It particularly relates to the conditioning of mineral surfaces to render the various minerals more amenable to electrostatic separation. Still more particularly the invention relates to conditioning mineral composites with anionic reagents and then subjecting the treated composite to electrostatic separation.

Refractory type minerals (i. e., those not easily susceptible to chemical attack) when in combination, such as kyanite-zircon, yield but slightly to electrostatic separation. Such separations are improved if the crushed mineral composite is deslimed or cleaned by dedusting or by moderate agitation with water. The introduction of acids such as hydrofluoric and sulfuric acids to the water during the desliming improves electrostatic separation somewhat; however, the degree of improvement frequently is not sufficient to warrant independent commercial application of the acids alone.

Accordingly, it is an object of this invention to provide a method whereby the surfaces of refractory mineral composites are conditioned with anionic reagents and the composite thereby rendered more amenable to electrostatic separation. Other objects and advantages will be apparent and in part hereinafter appear.

These objects and advantages are accomplished in accordance with the invention by heating and drying a ground and deslimed mineral composite, thereafter treating said hot dry composite with a selective surface conditioning reagent, and then subjecting the conditioned composite to electrostatic separation whereby the selectively conditioned constituent is rendered more or less susceptible to the influence of an electrical potential differential than the unconditioned constituent; and thereby rendering said composite more amenable to electrostatic separation.

Suitable mineral composites adaptable for use in accordance with the present invention include those mineral composites having constituents which are not readily susceptible to chemical attack, hereinafter termed refractory. The separation of such composites as kyanite-zircon, sillimanite-quartz, kyanite-quartz, and the like, has

been found to be greatly improved by surface conditioning treatment in accordance with this invention.

In the present process the heating and drying of the mineral composite can be suitably accomplished by any heating and drying means generally adapted to such operations.

Suitable surface conditioning reagents for purposes of this invention include organic compounds which exhibit anionic and cationic characteristics. The presently preferred anionic conditioning agents are those having the following general structural formula:

15

 $R(COOH)_n$ 

wherein R is a normal, branched or cyclic hydrocarbon appendage, and n is any whole number consistent with the nature of R. Such substances include normal aliphatic acids such as heptylic acid, propionic acid, acetic acid, mixed coconut fatty acids, crotonic acid, oleic acid and the like; dibasic acids such as fumaric acid and the like; aryl acids such as benzoic acid, the naphthenic acids, salicyclic acid, phthalic acid, cresylic acid, and the like; and other organic compounds having acid properties and a hydrocarbon appendage of sufficient length. Although cresylic acid has a hydroxyl group instead of a carboxyl, the hydroxyl group attached to an aryl appendage exhibits acid properties.

In operation the mineral composite is first crushed to a degree which will substantially liberate the various mineral constituents from one another. This can be accomplished by any suitable materials disintegrating means. The ground

material is thereafter mixed with water or other suitable suspending medium to form a pulp containing about 50 to 70 per cent solids and then deslimed. The desliming can be accomplished by

treating the pulp with about 0.05 to 50 pounds of at least one mineral acid per ton of composite in the pulp. Mineral acids such as hydrochloric, hydrofluoric, nitric, phosphoric, sulfuric, sulfurous and the like have been found to be satisfactory for this purpose. Mixtures of hydrofluoric acid or fluoride salts with other acids, such as sulfuric, have also been found to be effective in this connection. When such mixtures are employed a few tenths of a pound of the hydrofluoric acid or fluoride and 1 to 50 pounds of sulfuric acid is generally sufficient.

The time for this initial desliming and surface cleaning treatment is not critical and will vary greatly with the nature of the mineral, the de-

gree of fineness of the crushed composite, the rate of agitation and other such factors. About one-half an hour has generally been found to be sufficient for agitation. The liquid phase is thereafter removed from the treated solids by suitable solid-liquid separating means such as sedimentation and decantation, filtration, centrifuging, and the like. Thereafter the deslimed composite is preferably washed with sufficient water to remove any liquids which may be entrapped in the mass. The dewatered composite is then dried. Any suitable method can be employed to dry the mineral composite. Merely heating or passing hot dry air through the mass has been found to dry the material satisfactorily.

Thereafter to each ton of the hot dry material about 0.05 to 5 pounds of an anionic reagent is added and intimately mixed therewith. The temperature of this conditioning treatment will vary somewhat with the reagent employed and the mineral being treated. In general temperatures between about 50 to 300 degrees centigrade, or temperatures sufficient to volatilize the reagent have been found satisfactory. The reagent can be added as a solid, liquid or gas. Some anionic reagents such as benzoic acid are sufficiently volatile so that they can be added in pure state without any danger of adding an excessive amount or of failing to get a uniform distribution of the reagent throughout the composite. Other less volatile reagents, such as the coconut fatty acids, can be added as solutions in suitable volatile solvents such as carbon tetrachloride, gasoline, kerosene, and the like, in order to achieve a greater control of the amount of reagent added and a greater uniformity of dispersion. The conditioning treatment can be accomplished by any of the many well known processes for intimately and uniformly blending small amounts of materials with larger amounts of crushed solid materials. For example, the hot dry material can be tumbled with the reagent for a sufficient time to insure a substantially uniform dispersion or contacting of the reagent and the material being treated. Thereafter the thus treated composite is immediately passed through an electrostatic separation.

The following examples will show more specifically how the invention may be carried out but it is not limited thereto.

#### EXAMPLE I

A ground kyanite-zircon composite was moderately agitated with four pounds of hydrofluoric acid per ton, in a 60 to 70 per cent solids pulp. The desliming liquid was removed by sedimentation and decantation. This was followed by washing the deslimed material several times with water and then dewatering by sedimentation and decantation. The material was dried by heating and agitating the mass; the hot dry material was then at the stage for the anionic reagent treatment. To separate batches of the hot dry deslimed composite anionic reagents were added and intimately blended by rolling and stirring the mixture. The reagents were added in a concentration equivalent to three pounds of reagent per ton of composite. The thus treated material was immediately passed through a single stage roll-type separator having a non-ionizing negative electrode adjacent to the roll. A partial summary of the results is given in Table I below. The "deflectant" is the fraction attracted toward the electrode, while the "residue" remains close to the roll.

4  
TABLE I

*Effect of various reagents on the kyanite-zircon separation*

| 5  | Test No. | Treatment          | Product    | Weight Percent | Zircon, per cent |                   |
|----|----------|--------------------|------------|----------------|------------------|-------------------|
|    |          |                    |            |                | Assay            | Fraction of Total |
| 10 | 1...     | None               | deflectant | 27             | 56               | 32                |
|    |          |                    | residue    | 73             | 43               | 68                |
|    |          |                    | composite  | 100            | 47               | 100               |
|    | 2...     | Benzoic acid       | deflectant | 28             | 66               | 63                |
|    |          |                    | residue    | 72             | 15               | 37                |
|    |          |                    | composite  | 100            | 29               | 100               |
|    | 3...     | Salicylic acid     | deflectant | 23             | 75               | 74                |
|    |          |                    | residue    | 77             | 8                | 26                |
|    |          |                    | composite  | 100            | 20               | 100               |
|    | 4...     | Phthalic Anhydride | deflectant | 26             | 48               | 65                |
|    |          |                    | residue    | 74             | 9                | 35                |
|    |          |                    | composite  | 100            | 19               | 100               |
|    | 5...     | Oxalic acid        | deflectant | 14             | 75               | 24                |
|    |          |                    | residue    | 86             | 40               | 76                |
|    |          |                    | composite  | 100            | 45               | 100               |
|    | 20       |                    | deflectant | 34             | 77               | 93                |
|    | 6...     | Heptylic acid      | residue    | 66             | 3                | 7                 |
|    |          |                    | composite  | 100            | 28               | 100               |
|    |          |                    | deflectant | 30             | 74               | 69                |
|    | 7...     | Cresylic acid      | residue    | 70             | 14               | 31                |
|    |          |                    | composite  | 100            | 32               | 100               |

25 From these results it can be seen that an improvement can be obtained by treatment with anionic reagents in general. The data also shows that oxalic acid, unlike the other reagents in having no hydrocarbon appendage, does not give any appreciable improvement in separation.

35 This process of conditioning with anionic reagents was extended to other combinations of minerals. The same conditioning process was used but the electrostatic separation was more elaborate, the separator had six stages instead of one as in Example I. The first three stages had negative electrodes with the non-deflectant passed through successive stages to yield a tailing. The deflectant from each of the three stages was 40 combined as heads for the second three stages. The second three stages had positive electrodes with the non-deflectant passed through successive stages to yield the concentrate. The deflectant from each of the three stages yields a middling fraction which may in some cases contain a third mineral component which is electrically conductive.

#### EXAMPLE II

50 A sillimanite-quartz composite was deslimed as in Example I. Some portions of the deslimed composite were not treated with any anionic reagent; and used as controls. Other portions were anionically conditioned as in Example I. The 55 materials were then subjected to electrostatic separation. The collected portions were assayed by a sink and float procedure in acetyline tetrabromide. The results are in part summarized in Table II.

60 TABLE II  
*Effect of benzoic acid on sillimanite-quartz separation*

|    | Treatment    | Weight Percent | Concentrate 2.96 Density Assay Per Cent Sink | Calculated Sillimanite Recovery Per Cent |
|----|--------------|----------------|----------------------------------------------|------------------------------------------|
| 65 | None         | 34.6           | 93.0                                         | 82                                       |
| 70 | Benzoic acid | 34.1           | 98.6                                         | 89                                       |

75 This shows an improvement in both grade and recovery by the use of benzoic acid as the conditioning reagent. Other anionic reagents had a similar effect.

**5**  
**EXAMPLE III**

Using the process of Example II on the kyanite-quartz mixture, the assay of the concentrates (kyanite) were approximately the same but the recoveries highly divergent. With benzoic acid the recovery was 90% and without benzoic acid, 78%; kyanite was apparently lost in the tailing. Table III gives an assay of several of the coarse sizes in the tailing.

**TABLE III**  
*Effect of benzoic acid on a kyanite-quartz separation*

| Treatment    | Per cent Kyanite Tail-ing Composition |             | Tailing Size Analysis Weight Per cent |             |
|--------------|---------------------------------------|-------------|---------------------------------------|-------------|
|              | -10+14 mesh                           | -14+20 mesh | -10+14 mesh                           | -14+20 mesh |
| None         | 27                                    | 9.3         | 4.1                                   | 13.2        |
| Benzoic acid | 3.7                                   | 0.5         | 3.7                                   | 10.2        |

In addition to improving the recovery of the kyanite, the benzoic acid enables the processing of coarser-sized material. It also counteracts sensitivity to high humidity weather conditions.

From the above description and examples, it is apparent that a definite improvement in the electrostatic separation of refractory mineral composites is obtained by the conditioning of the mineral surfaces with anionic reagents.

While the invention is particularly described in connection with a conditioning treatment with anionic reagents such as benzoic acid, phthalic acid, heptylic acid and the like, it is not limited thereto, certain basic reagents such as the amines also function in a similar manner.

Since many widely differing embodiments of the invention will occur to one skilled in the art, the invention is not limited to the specific details illustrated and described, and various changes may be made therein without departing from the spirit and scope thereof.

What is claimed is:

1. In a process for the electrostatic separation

**6**

of the liberated and deslimed constituents of a mineral composite of a type resistant to chemical attack and of the class consisting of kyanite-zircon, sillimanite-quartz, and kyanite-quartz, which involves electrostatic separation of the composite constituents, the steps prior to said separation which comprise heating and drying said composite and then treating said hot dry composite with about 0.05 to 5 pounds of an organic anionic conditioning agent per ton of composite, said conditioning agent being a carboxylic acid having a hydrocarbon appendage, whereby at least one of said composite constituents is selectively filmed with said conditioning agent and said composite constituents are thereby rendered more amenable to electrostatic separation.

2. The process of claim 1 wherein the anionic conditioning agent is of the group of compounds having the formula



wherein: R is a normal, branched, or cyclic hydrocarbon appendage and n is any whole number consistent with the chemical nature of R.

FOSTER FRAAS.

**REFERENCES CITED**

The following references are of record in the file of this patent:

| UNITED STATES PATENTS |                 |               |
|-----------------------|-----------------|---------------|
| Number                | Name            | Date          |
| Re. 3,677             | Bureau of Mines | Dec. 1942     |
| 959,646               | Swart           | May 31, 1910  |
| 35 2,090,418          | Johnson         | Aug. 17, 1937 |
| 2,105,826             | Tartaron        | Jan. 18, 1938 |
| 2,154,682             | Johnson         | Apr. 18, 1939 |
| 2,197,865             | Johnson         | Apr. 23, 1940 |
| 2,198,972             | Peddrick        | Apr. 30, 1940 |
| 40 2,245,200          | Johnson         | June 10, 1941 |

OTHER REFERENCES

Fraas and Ralston, Electrostatic Separations of Solid, Industrial and Engineering Chemistry, vol. 32, No. 5, pages 600 to 644.